

# United States Patent [19]

Downing

[11] Patent Number: 4,961,458

[45] Date of Patent: \* Oct. 9, 1990

[54] **METHOD OF FORMING A DIE CASTING WITH COATED EXPENDABLE CORES**

[75] Inventor: Robert E. Downing, Toledo, Ohio

[73] Assignee: Farley, Inc., Chicago, Ill.

[\*] Notice: The portion of the term of this patent subsequent to Sep. 19, 2006 has been disclaimed.

[21] Appl. No.: 374,649

[22] Filed: Jun. 30, 1989

**Related U.S. Application Data**

[63] Continuation-in-part of Ser. No. 319,543, Mar. 6, 1989, Pat. No. 4,867,225, which is a continuation-in-part of Ser. No. 173,558, Mar. 23, 1988, abandoned.

[51] Int. Cl.<sup>5</sup> ..... B22C 1/22; B22C 3/00;  
B22C 9/10

[52] U.S. Cl. ..... 164/72; 164/113;  
164/138; 164/369; 164/527; 427/134; 523/139;  
523/148

[58] Field of Search ..... 164/369, 72, 113, 138,  
164/527; 427/134; 523/139, 148

[56] **References Cited**

**U.S. PATENT DOCUMENTS**

- |           |         |               |           |
|-----------|---------|---------------|-----------|
| 3,922,245 | 11/1975 | Skubon et al. | 427/134 X |
| 4,001,468 | 1/1977  | Skubon et al. | 427/134   |
| 4,096,293 | 6/1978  | Skubon et al. | 427/134   |
| 4,194,915 | 3/1980  | Perkins       | 427/134 X |

4,413,666 11/1983 Page ..... 164/72  
4,529,028 7/1985 Dybala et al. ..... 164/138 X  
4,766,943 8/1988 Page ..... 164/72  
4,867,225 9/1989 Downing ..... 164/369

*Primary Examiner*—Richard K. Seidel

*Assistant Examiner*—J. Reed Batten, Jr.

*Attorney, Agent, or Firm*—Hugh Adam Kirk

[57]

**ABSTRACT**

A method for producing high pressure die castings with undercut regions comprises forming an expendable coated core of specific composition, placing it in the die in a die casting machine, injecting molten metal into the die to form the casting and separating the casting from the die and the core from the casting. The composition of the expendable coated core comprises a base sand core held together by a resin binder; a first, bottom, hard refractory coating comprising fused silica and a refractory binder containing at least two of the following additives: a suspension agent, a dispersant, a wetting agent, and an anti-skimming agent; and a second, top, soft, or release coating containing a release material selected from the group consisting of anhydrous powdered aluminum, graphite, talc, titanium dioxide and zircon, and a resinous binder containing at least two different compounds selected from the group of additives consisting of a suspension agent, a dispersant, and an anti-settling agent.

3 Claims, No Drawings

**METHOD OF FORMING A DIE CASTING WITH  
COATED EXPENDABLE CORES**

**RELATED PATENT AND PATENT  
APPLICATION**

This application is a continuation-in-part of copending Application Ser. No. 319,543 filed Mar. 6, 1989, which in turn is a continuation-in-part of Application Ser. No. 173,558 filed Mar. 23, 1988, now abandoned. The Application Ser. No. 319,543 is now U.S. Pat. No. 4,867,225 issued Sept. 19, 1989 and is directed to the coated core used in this invention.

**BACKGROUND OF THE INVENTION**

This application is an improvement in die casting sand cores and core coatings disclosed in applicant's assignee's U.S. Pat. Nos. 4,413,666 issued Nov. 8, 1983 and No. 4,766,943 issued Aug. 30, 1988 to Enno H. Page and U.S. Pat. No. 4,529,028 issued July 16, 1989 to 20 Dybala and Maczko.

There are many patents on processes for producing die castings and dies using expendable cores with various compositions of coatings for the dies and the cores therefor to withstand the hot metals poured or injected 25 into the dies until the metal are solidified. Even applicant's assignee owns the above mentioned related patents and patent applications which disclose expendable sand cores having coatings, which cores have good shake-out properties, good wash-out resistance, good 30 resistance to surface penetration, good shelf life, and high core strength to withstand pressures in excess of 1000 psi to from smooth undercut regions in die castings.

Nevertheless, still higher pressures in die casting processes are often desired and therefore it is essential to increase the strength of the expendable cores used 35 therein. Applicant, after considerable experimenting and testing, has unexpectedly discovered new compositions and additives for the coatings of such expendable sand cores for die casting dies, which coated cores have improved physical properties over what has been known before; namely to withstand greater pressures and hotter metal melts, and to produce better and smoother undercut portions in die castings.

**OBJECTS AND ADVANTAGES**

Accordingly, it is an object of this invention to provide a new process for producing die castings by means of an improved expendable coated sand core for die casting dies, which cores are stronger than the coated expendable cores disclosed in the known prior art.

Another object is to provide a process to produce die casting dies with cores having coatings for expendable sand cores for die casting dies, which cores will withstand pressures up to about 14,000 pounds per square inch.

Another object is to produce improved die castings and dies by a process using coated expendable sand cores, which coatings adhere better and penetrate further into the sand grains on the surface of the cores to produce a stronger shell and a harder surface on the cores than previously known coatings, and which coatings resist cracking and resist penetration and thermal deterioration by the hot metal injected into the dies.

Still another object is to provide a process to produce a die and die casting therefrom by using an expendable die casting core which forms in die castings undercut

regions with smoother undercut surfaces than previously known.

A further object is to improve the quality of the liquid suspensions of coatings for expendable sand cores used in the above process, which liquid suspensions have a greater stability, a better shop life, and do not evaporate like the prior known coatings as disclosed in applicant's assignee's above mentioned patents and applications.

Still a further object is to produce coated expendable sand cores which separate more easily from the final die cast casting than has been obtained with the coatings disclosed in applicant's assignee's above mentioned patents and patent applications.

**SUMMARY OF THE INVENTION**

The method or process of this invention comprises the steps of producing a die casting in a high pressure die casting die, which casting has undercut regions formed by an expendable core with specific coatings to withstand the pressures and temperatures of the molten metal in the die and still be able to remove the core easily from the die or mold after the coating has solidified in the die. The molten metal usually is aluminum and/or its related alloys. Thus the steps of this invention comprise forming such a coated core, placing the core in the die casting die to form the die for the undercut casting to be formed therein, closing the die, injecting the molten metal into the die, permitting the molten metal to solidify in the die and its heat to deteriorate and disintegrate the core, opening the die, removing the casting and core from the die, and separating the disintegrated core from the casting, such as by shaking. By disintegrated, I mean that the resinous binder, for the sand grains forming the base of the core, is deteriorated or decomposed by the heat of the molten metal so that the core breaks up or crumbles into particles of sand grains which can easily be removed from the final casting.

The specific expendable core used in the process of this invention to produce the die and casting therefrom comprises a sand core with two improved coatings, a first, base, hard refractory coating and a second, top, soft release coating.

The expendable core is preferably formed of silica sand placed in a mold so that each sand grain is in contact with an adjacent sand grain, and the sand grains are bound together by a resin oxidized in the mold.

This sand core is then dipped or sprayed with an aqueous suspension comprising the first, base, hard refractory coating for the core, which aqueous suspension contains finely ground fused silica as its primary and major refractory material, but which may also contain a minor amount of other refractory oxides. These refractory materials have particle sizes less than about 100 microns and an average particle size of less than about 50 microns so as to be easily suspended in an aqueous solution. This first coating aqueous suspension also includes less than about 15% by weight of a binder for these particles which is a refractory material and comprises colloidal silica. Particles of the refractory and binder are maintained in this aqueous suspension by the addition of less than 1.5% and usually less than about 1% by weight of the aqueous suspension of two different compounds or additives selected from the groups of additives consisting of (1) a suspension agent (2) a dispersant, (3) a wetting agent, and (4) an anti-skinning agent. These four additives may act, respectively, also

60  
55  
60  
65

as a thickening agent, as a deflocculent, to reduce surface tension, and to reduce water evaporation. These agents not only improve the shelf life of the aqueous suspension, but also unexpectedly improve the quality of the coating, and as a result thereof, an improved surface on the undercut region in the final die cast product. In this composition the amount of water in this first coating aqueous suspension is critical for the proper effect of the additives, that is the water content is at least 12% and not more than 30% by weight of the whole mixture suspension.

After the first, base, or refractory coating is dried on the sand core, the second, top soft release coating is applied by either dipping or spraying, which second coating liquid suspension comprises primarily solid particles of a release material selected from a group consisting of powdered aluminum, graphite, talc, titanium dioxide, and zircon, suspended in a non-aqueous solvent, such as for example isopropyl alcohol. The particle size of the release material solids are less than about 100 microns and preferably having an average particle size of less than about 40 microns. This solvent or liquid comprises at least 30% and up to 90% by weight of this second coating liquid suspension. In order to insure a uniform suspension of the particles of release material in this organic solvent, there is added less than about 10% by weight of a resinous binder, preferably a thermoplastic resin, and less than about 15% of at least two different compounds or additives selected from the groups of additives consisting of: (1) a suspension agent of an aluminum silicate compound (similar to the suspension agent employed in the first coating aqueous suspension), (2) a dispersant, and (3) an anti-settling agent.

When this second or release coating has dried, the coated core is then ready for placement into the die casting die for production of a casting with an undercut region formed by this coated core.

#### DETAILED DESCRIPTION OF PREFERRED EMBODIMENTS

##### I.

###### The Process

A process for producing the undercut die casting in a high pressure die casting die comprises the following steps:

1. The first step in producing a die casting with undercut regions according to this invention is to produce the core for forming these undercut regions. This core is produced by first forming the base thereof by mixing sand with a binder and forming it to the form of the core desired and letting it solidify in that form.
2. Then the solidified core is coated with a base refractory aqueous coating.
3. After this aqueous coating has dried on the core, the core is then coated with a top release organic coating.
4. After this second coating has dried, the core is placed into the mold or die of the die casting machine. The specific compositions of the core and its two coatings are described below.
5. After the core is placed in the die casting die, the die is closed and the hot metal is injected under high pressure into the mold to form the casting.
6. The die is remained closed until the molten metal has solidified and its high temperature has disintegrated the core.

7. The die then is opened and the solidified casting and core are removed, and the core is separated from the die casting, such as by shaking.

##### II.

###### The Specific Core Compositions

###### A. Sand Base Core

The composition of the sand base core may be a white silica washed spherical grain sand having a low acid value and a neutral pH, that is between 6 and 8. These sand particles are blown into a mold and bound together by a binder which comprises between about 0.7 and 5% by weight of the sand. If this binder is a furan resin it may range between about 0.75 and 2.5% by weight of the sand, and preferably between about 1 and 2%, and more preferably between about 1.3 and 1.7% by weight of the sand. This furan resin is cured in situ in the mold with sulfur dioxide gas. The binder also may contain between about 2 and 20% by weight of the binder of silane, preferably between about 3.5 and 15% and more preferably between about 5 and 10% by weight of the furan resin. This furan resin also contains methyl ethyl ketone peroxide in an amount between about 40 and 70% by weight of the binder, and preferably between about 50 and 60%, and more preferably about 55% by weight of the binder. Thus, this base sand core is similar in composition to that disclosed in the above mentioned related patents and patent application assigned to applicant's assignee.

###### B. The First, Base Hard Refractory Coating

The composition of the aqueous suspension which forms the first, base hard refractory coating on the sand core comprises primarily fused silica ground so that all the particle sizes are less than 100 microns, with an average particle size of less than about 50 microns. This refractory comprises between about 40 and 85% and preferably between about 64 and 85% by weight of the aqueous coating, and of this refractory the fused silica ranges between about 40 and 80% by weight of the aqueous suspension. In the grinding of this fused silica there is obtained less than about 15% of colloidal silica and usually less than about 10%, that is of less than about 1 micron in size, which colloidal silica acts as a binder for the particles in the final coating, but more colloidal silica may be added, if desired. However, a minor percentage of the solids in the final coating may comprise similar micron sized particles of other refractory oxides, such as alumina, zirconia and kaolin, which may range from 0% up to less than about 50% by weight of the aqueous suspension, and correspondingly a minor percentage of these other refractory particles in the coating. However, coatings without any other refractory oxides than fused silica therein have been found to be very satisfactory.

To this aqueous suspension of refractory and binder particles there are added less than about 1.5% by weight of aqueous suspension of at least two different compounds or additives from the following four groups of additives or agents, namely:

- (1) The first additive, namely a suspension agent, in this instance acts more as a thickener or thickening agent and comprises a clay derivative or aluminum silicate compound, such as for example "Bentone" which is an aminated bentonite, smectite, or hectorite. The percentages of this suspension agent ranges up to about 1% by weight of the aqueous suspension.

- (2) The dispersant which acts as a deflocculant or a dispersing agent is added in an amount less than 1.5% and preferably less than about 0.8% by weight of the aqueous suspension. This agent may comprise an alkali phosphate and/or poly acrylate, including a poly methacrylate, which promotes and maintains the separation of the individually extremely fine particles of solids of refractory in the suspension and prevents their flocculation. 5
- (3) The wetting surfactant agent improves the dispersing of the particles in the liquid by reducing the surface tension when dissolved in water, such as causing the water to penetrate more easily into or to be spread over the surface of the particles in the suspension. An effective wetting agent includes compounds having acid and hydroxyl radicals such as a tertiary acetylene diol. The percentage of the wetting agent is less than about 0.5% and preferably less than 0.1% by weight of the aqueous suspension. 10
- (4) The anti-skimming agent prevents evaporation of water from the composition and may comprise a high aliphatic alcohol of 8 or more carbon atoms. The percentage of anti-skimming agent is less than about 0.1% by weight of the aqueous suspension. 15

After the core has been coated with this aqueous suspension of the first coating and dried, this hard coating has a thickness of between about 25 and 2000 microns, and preferably between about 100 and 750 microns (0.004 and 0.030 inches) and more preferably between about 150 and 500 microns (micrometers) 20 (0.006 and 0.020 inches). 25

#### C. The Second, Top, Soft Release Coating

The core with its dried first coating is then coated with the liquid suspension of the second soft coating which comprises primarily solid particles of one or more release materials selected from the group consisting of anhydrous aluminum powder, graphite, talc, titanium dioxide, and zircon, which materials are suspended in an organic solvent, such as isopropyl alcohol. These solid particles of release materials have a particle size of less than about 100 microns and an average particle size of less than about 40 microns. The percentage of these release material particles in the suspension ranges between about 5% and 60% by weight of the whole suspension for the heavier particles like titanium dioxide 40 and zircon, and only up to about 40% by weight of the lighter particles like anhydrous aluminum, graphite and talc. 45

In order to bind together the particles of the release material in the final coating, there is added to the second liquid suspension a resinous binder, such as a dark brittle high melting point aliphatic hydrocarbon insoluble thermoplastic resin or a phenolic resin, in an amount between about 0.2 and 10% and preferably between about 1% and 5% by weight of the liquid suspension. 6

In addition to the release materials and binder in this outer or top coating, there are also added less than about 15% by weight of the liquid suspension of at least two different compounds or additives from the groups of additives consisting of (1) a suspension agent, (2) a dispersant, and (3) an anti-settling agent. The suspension agent may be similar to that employed in the first coating, namely a clay derivative composition or aluminum silicate compound, including clays, "Bentone", bentonite, kaolin, and the like. The amount of the suspension agent is less than about 10% by weight of the liquid suspension. The dispersant may be a phosphate, polycarbonate or sulfonate and added in an amount up to about 4% by weight of the liquid suspension. The anti-settling agent may be a methoxy propylamine and may be added up to an amount of about 3% by weight of the liquid suspension. 10

In the second or release coating, the non-aqueous or organic liquid is generally a major portion of the suspension composition, namely ranging between about 30 and 90% by weight of the liquid suspension including the solids therein. 15

When the second and soft coating is dried on the first coating on the core, the thickness of this second coating is usually less than that of the first coating and ranges between about 15 and 2000 microns and preferably between about 25 and 750 microns (0.001 and 0.030 inches) and more preferably between about 50 and 200 microns (0.002 and 0.008 inches). Since this top coating is softer than the first coating, it can be compressed by the pressure of the hot metal flowing against it, and accordingly can be made thicker than the hard base coating, if desired. 20

#### D. Specific Examples

The following Table 1 is of six different compositions of the aqueous first, base, hard refractory coating that have been used on sand cores of the specific composition mentioned above, which coatings have produced successful cores and die castings with undercut portions:

TABLE I

| FIRST COATING SUSPENSION COMPOSITION |           |           |           |           |           |           |
|--------------------------------------|-----------|-----------|-----------|-----------|-----------|-----------|
| Ingredients in Percentage by Weight  | Example 1 | Example 2 | Example 3 | Example 4 | Example 5 | Example 6 |
| <u>Refractories 40-85%</u>           |           |           |           |           |           |           |
| Fused Silica 40-80%                  | 50.67     | 73.00     | 69.30     | 60.17     | 60.57     | 65.34     |
| Alumina 0-50%                        |           |           |           | 15.11     | 14.76     |           |
| Zirconia 0-50%                       | 25.5      |           |           |           |           |           |
| Kaolin 0-15%                         |           |           |           |           |           | 10.9      |
| <u>Binder 1-15%</u>                  |           |           |           |           |           |           |
| Colloidal Silica                     | 5.63      | 8.09      | 7.70      | 9.01      | 9.03      | 9.16      |
| <u>Additives .1-1.5%</u>             |           |           |           |           |           |           |
| (1) Suspension Agent 0-1%            |           |           |           |           |           |           |
| Amine-treated Bentonite ("Bentone")  | 0.20      | 0.20      | 0.50      |           | 0.20      |           |
| (2) Dispersant 0-1.5%                |           |           |           |           |           |           |
| Alkali Polyacrylate                  |           |           |           | 0.10      | 0.20      | 0.20      |
| Alkali Phosphate                     | 0.30      |           | 0.10      |           |           |           |
| (3) Anti-skimming Agent 0-1%         |           |           |           |           |           |           |
| More than 8 carbon atom alcohol      |           | 0.05      |           | 0.01      |           |           |
| (4) Wetting Agent 0-5%               |           |           |           |           |           |           |
| Tertiary Acetylene Diol              |           | 0.05      |           |           |           |           |
| Water 12-30%                         | 17.7      | 18.60     | 22.40     | 15.60     | 15.24     | 14.40     |

The second, top, soft release coatings were produced according to the five examples in the following Table II and were applied to the first coatings in the Examples 1 through 6 in Table I above, and successful results were obtained therefor both in the production of the coated cores and in the final castings with smooth undercut regions.

(E) separating said casting from said core by shaking the disintegrated core from said solid casting.

2. A method for forming a die casting having an undercut region having a smooth and lustrous surface, the steps comprising:

(A) forming a die casting die having a casting surface that includes at least one expendable sand core that

TABLE II

| SECOND COATING SUSPENSION COMPOSITION |           |           |           |           |           |
|---------------------------------------|-----------|-----------|-----------|-----------|-----------|
| Ingredients in Percentages by Weight  | Example 1 | Example 2 | Example 3 | Example 4 | Example 5 |
| <u>Release Materials 5-60%</u>        |           |           |           |           |           |
| Anhydrous Powdered Aluminum 0-30%     |           | 12.2      |           | 12.7      |           |
| Graphite 0-40%                        | 28.5      |           | 28.5      |           |           |
| Talc                                  |           | 13.1      |           |           |           |
| Titanium Dioxide 0-40%                |           |           |           | 25.0      |           |
| Zircon 0-60%                          |           |           |           | 9.1       |           |
| <u>Binder .2-10%</u>                  |           |           |           |           |           |
| Phenolic Resin 0-5%                   | 1.5       |           |           |           |           |
| Thermoplastic Resin 0-5%              |           | 1.7       | 2.0       | 1.8       | 1.5       |
| <u>Additives .05-15%</u>              |           |           |           |           |           |
| (1) Suspension Agent 1-10%            |           |           |           |           |           |
| “Bentone”                             | 4.3       | 2.6       | 4.3       | 2.7       | 4.2       |
| (2) Dispersant .05-4%                 |           |           |           |           |           |
| Phosphate Ester/Sulfonate             | 0.5       |           | 0.5       |           | 0.5       |
| Polycarbonate                         |           | .1        |           | .1        |           |
| (3) Anti-settling Agent 0-3%          |           |           |           |           |           |
| Methoxy Propylamine                   | 1.2       |           | 1.2       |           | 1.2       |
| Solvent 30-90%                        |           |           |           |           |           |
| Isopropyl Alcohol                     | 64.0      | 70.3      | 63.5      | 73.6      | 67.6      |

While there is described above the principles of this invention in connection with specific process, products, apparatus and compositions, it is to be clearly understood that this description is made only by way of example and not as a limitation to the scope of this invention. 35

I claim:

1. A method for forming a die casting having an undercut region with a smooth and lustrous surface, the steps comprising:

(A) forming a die casting die having a casting surface 40 that includes at least one expendable sand core that forms said undercut region, said sand core consisting essentially of:

(1) a base of sand having grains that touch each other with the spaces between the grains being at 45 least partially filled with a resin binder;

(2) a first aqueous coating on said base consisting essentially of:

(a) at least about 40% by weight of said first coating of a refractory comprising fused silica 50 having a particle size of less than about 100 microns and an average particle size of less than about 50 microns;

(b) at least 1% and less than about 15% by weight of said first aqueous coating of a 55 binder; and

(c) at least 0.1% and less than about 1.5% by weight of said first aqueous coating of at least two different additives selected from the groups of additives consisting of: suspension 60 agents, dispersants, wetting agents, and anti-skimming agents; and

(3) a second liquid release coating;

(B) injecting molten metal into said die;

(C) permitting said metal to solidify to form said casting around said core and to disintegrate the base of said core;

(D) removing said casting and core from said die; and

forms said undercut region, said sand core consisting essentially of:

(1) a base of sand having grains that touch each other with the spaces between the grains being at least partially filled with a resin binder;

(2) a first aqueous refractory coating on said base;

(3) a second liquid release coating on said first refractory coating consisting essentially of:

(a) solid release particles having a particle size less than 100 microns and an average particle size of less than about 40 microns selected from the group consisting of anhydrous powdered aluminum, graphite, talc, titanium dioxide and zircon;

(b) between about 0.2 and 10% by weight of said second liquid coating of a resinous binder;

(c) between about 0.5 and 15% by weight of said second liquid coating of at least two different additives selected from the groups of additives consisting of a suspension agent, an anti-settling agent, and a dispersant;

(d) at least about 30% by weight of an organic solvent;

(B) injecting molten metal into said die;

(C) permitting said molten metal to solidify to form said casting around said core and to disintegrate the base of said core;

(D) removing the casting and core from said die; and

(E) separating said casting from said core by shaking the disintegrated core from said solid casting.

3. A method for forming a die casting having an undercut region having a smooth and lustrous surface, the steps comprising:

(A) forming a die casting having a casting surface that includes at least one expendable sand core that forms said undercut region, said sand core consisting essentially of:

- (1) a base of sand having grains that touch each other with the spaces between the grains being at least partially filled with a resin binder;
- (2) a first aqueous coating on said base consisting essentially of:
  - (a) at least about 40% by weight of said first coating of a refractory material comprising fused silica having a particle size of less than about 100 microns and an average particle size of less than about 50 microns;
  - (b) at least 1% and less than about 15% by weight of the first aqueous coating of a binder;
  - (c) at least 0.1% and less than about 1.5% by weight of said first aqueous coating of at least two additives selected from the groups of additives consisting of: a suspension agent, a dispersant, a wetting agent, and an anti-skinnning agent;
- (3) a second liquid release coating on said first aqueous coating consisting essentially of:
  - (a) solid release particles have a particle size less than 100 microns and an average particle size

5

10

15

20

25

30

35

40

45

50

55

60

65

less than about 40 microns selected from the group consisting of: anhydrous powdered aluminum, graphite, talc, titanium dioxide and zircon;

- (b) between about 0.2 and 10% by weight of said second liquid coating of a resinous binder;
- (c) between about 0.05 and 15% by weight of said release coating of at least two additives selected from the group of additives consisting of a suspension agent, an anti-settling agent, and a dispersant; and
- (d) at least about 30% by weight of an organic solvent;

(B) injecting molten metal into said die;

(C) permitting said molten metal to solidify to form said casting around said core and to disintegrate the base of said core;

(D) removing said casting and core from said die; and

(E) separating said casting from said core by shaking the disintegrated core from said solid casting.

\* \* \* \* \*

UNITED STATES PATENT AND TRADEMARK OFFICE  
CERTIFICATE OF CORRECTION

PATENT NO. : 4,961,458

DATED : October 9, 1990

INVENTOR(S) : Robert E. Downing

It is certified that error appears in the above-identified patent and that said Letters Patent is hereby corrected as shown below:

Col. 1, line 26, change "metal" to - - metals - - .  
Col. 1, line 33, change "from" to - - form - - .  
Col. 2, line 33, change "I mean" to - - is meant - - .  
Col. 7, line 65, change "soldify" to - - solidify - - .  
Col. 8, line 65, after "casting" (first occurrence) insert - - die - - .  
Col. 9, lines 18-19, change "skinning" to - - skimming - - .

Signed and Sealed this

Thirty-first Day of March, 1992

*Attest:*

HARRY F. MANBECK, JR.

*Attesting Officer*

*Commissioner of Patents and Trademarks*